

## UNITED STATES PATENT OFFICE

ALAN KISLOCK, OF FOREST HILLS, NEW YORK

## PROCESS OF MAKING CALCIUM MOLYBDATE

No Drawing.

Application filed November 6, 1926. Serial No. 146,849.

The invention relates to a novel and useful process for producing calcium molybdate, such for example as is used as an addition agent in the manufacture of alloy iron or steel.

5 Certain objects and advantages of the invention are set forth hereinafter, and others will be apparent herefrom to those skilled in the art, or may be ascertained by practicing 10 the invention. The invention consists in the novel steps, sequences of steps, and processes hereinafter described.

By my invention I produce calcium molybdate, suitable for an addition agent in the 15 manufacture of alloy iron and steel, from commercially-available materials by primary elimination of deleterious agents or ingredients, such as sulfur, and subsequent reaction of a molybdenum oxide with an oxide of calcium. I preferably effect this primary purification as a step in a continuous process comprising the production of the molybdenum oxide from an ore or ore concentrate and the 20 subsequent production of the calcium molybdate as a final product of the process. This latter feature, however, is optional in so far as concerns the broader aspects of the invention.

The usual or commercially available sources 25 of molybdenum-bearing ores seldom carry more than one per cent of the mineral. Such ores are usually converted, as by the well-known flotation process, into a concentrate carrying approximately eighty or ninety per 30 cent of molybdenum sulfide. This concentrate is the usual starting point for the manufacture of any of the marketable forms of molybdenum, such for instance as the calcium molybdate already referred to. The process 35 of my present invention is well adapted to utilize as the initial material this molybdenum sulfide concentrate, as produced from the ore by present commercial practice.

Molybdenum sulphide is the raw material 40 most available as a starting point for the manufacture of all forms and compounds of molybdenum. In its natural state there are often associated with it other minerals or metallic compounds, such as sulfides of iron, 45 copper, etc. The first step in the process of

manufacture involves a concentration of the crude and usually low-grade molybdenum sulfide ore into a high grade molybdenum-sulfide concentrate. In the concentration of the crude molybdenum sulfide ore, ordinarily 55 by flotation process, the impurities, such as iron and copper sulfides, etc., which may be present in the original ore are often likewise concentrated, unless they be separated therefrom by several chemical methods well known 60 in the art of flotation. Such separations however are seldom entirely efficient, so that in the usual commercial molybdenum sulfide concentrates may be found at least minor percentages of the impurities above men- 65 tioned.

Since this is true, a commercially satisfactory process of making calcium molybdate from molybdenum sulfide concentrates must be capable of being carried out even though 70 such minor amounts of impurities be retained.

These impurities often result in the production of a final calcium molybdate containing an amount of sulfur sufficient to prevent 75 the use of the calcium molybdate in the production of high grade alloy steels, whereas I have found that if the oxidation of the molybdenum sulfide is substantially completed prior to the introduction of the calcium 80 oxide, hydroxide, or carbonate, these impurities do not interfere with the production of a substantially sulfur-free calcium molybdate and without any appreciable loss of molybdenum. 85

As is well known, sulfur is detrimental to the manufacture of high-grade iron and steel, and the elimination thereof during the process of conversion of the raw material is not only usually desirable, but in many cases 90 is absolutely necessary. Accordingly, my invention, in certain aspects thereof, is directed toward effecting the simple, efficient and economical elimination of the sulfur from the concentrates prior to the formation of the 95 calcium molybdate.

In order to effect and realize these objects and advantages, I preliminarily subject the concentrated molybdenum sulfide to an oxidizing roast, whereby the sulfur recombines 100

and is entirely driven off, and the purified concentrate is thereafter converted gradually into molybdenum trioxide. By intermixing calcium oxide with the molybdenum trioxide, and applying sufficient heat, calcium molybdate may be produced according to the following reaction:—



- 10 In practice I prefer to effect this reaction in the same furnace in which the molybdenum sulfide is roasted to the trioxide, and as a continuing process therewith. In accordance with this feature of the invention, the calcium oxide is introduced in proper proportion, and at a point in the progress of the concentrates through the roasting furnace beyond that where the sulfur has been eliminated therefrom, and by obtaining or raising 15 the temperature at this point sufficiently to effect the desired reaction.

At this point in the roasting of the molybdenite, namely after the elimination of the sulfur, calcium hydrate is fed into the 20 roasting furnace at a rate which synchronizes with the feed of the molybdenum sulfide, and in such quantity that the ratio of calcium oxide to molybdenum-trioxide is substantially as 1:2.57, which satisfies the 25 formula  $\text{CaMoO}_4$  and the reaction already stated.

After the oxide of molybdenum and the lime become thoroughly mixed in the furnace, the temperature is raised sufficiently to 30 bring about the desired reaction, the temperature being usually raised in practice to approximately 1400° F. at which point the union becomes complete, and the resulting calcium molybdate is delivered directly from 35 the ore roasting furnace.

In commercial work my process may be satisfactorily carried on by using a multiple hearth ore roasting furnace. I preferably employ a gravity operating furnace of this 40 type. In that case the calcium hydrate is fed into one of the lower hearths, prior to which the sulfur has been entirely driven off. The feeding mechanism has preferably variable speed control to regulate the feeding 45 speed of the calcium hydrate. Additional heating means are provided, when required, to raise the temperature sufficiently to cause the materials on the hearths to react to produce the calcium molybdate as the final product of the continuous furnacing operation.

By my process calcium molybdate substantially free from sulfur is produced with less 50 difficulty, greater efficiency and more economy than by the processes heretofore in use.

It will be understood that the procedure and practice in carrying out my invention 55 may be varied, and in some respect quite widely, from the preferred manner of per-

forming the principal step, and the other steps as well, of my process without departing from the principles of the invention and without sacrificing its chief advantages.

What I claim is:—

1. The process of making calcium molybdate which comprises roasting molybdenum sulfide to produce molybdenum trioxide and mixing calcium oxide with the molybdenum trioxide and applying additional heat thereto to cause them to combine to produce calcium molybdate. 70

2. The process of making calcium molybdate which comprises roasting molybdenum sulfide to produce molybdenum trioxide and mixing calcium oxide with the molybdenum trioxide and applying additional heat to a temperature of approximately 1400 degrees Fahrenheit thereto to cause them to combine to produce calcium molybdate. 75 80

3. The process of making calcium molybdate which comprises oxidizing molybdenum sulfide to molybdenum trioxide and as a step subsequent to the elimination of the sulfur applying additional heat and effecting a reaction of the molybdenum trioxide with calcium oxide to produce calcium molybdate. 85 90

4. The process of making calcium molybdate which comprises oxidizing molybdenum sulfide to molybdenum trioxide and as a step subsequent to the elimination of the sulfur raising the temperature to approximately 1400 degrees Fahrenheit and effecting a reaction of the molybdenum trioxide with calcium oxide to produce calcium molybdate. 95 100

5. The process of making calcium molybdate which comprises progressing molybdenum sulfide through a roasting furnace to convert it to molybdenum trioxide, and at a point after the molybdenum sulfide has been completely converted to molybdenum trioxide feeding in a calcium oxide at a proportional rate, and effecting a reaction to produce calcium molybdate as the final product of the furnacing operation. 105

6. The process of making calcium molybdate which comprises progressing molybdenum sulfide through a roasting furnace to convert it to molybdenum trioxide, and at a point after the molybdenum sulfide has been completely converted to molybdenum trioxide feeding in a calcium oxide at a proportional rate, and applying additional heat thereto and effecting a reaction to produce calcium molybdate as the final product of the furnacing operation. 110 115

7. The process of making calcium molybdate which comprises progressing molybdenum sulfide through a roasting furnace to convert it to molybdenum trioxide, and at a point after the molybdenum sulfide has been completely converted to molybdenum trioxide feeding in a calcium oxide at a proportional rate, and raising the heat of the furnace to approximately 1400 degrees Fahrenheit and 120 125 130

effecting a reaction to produce calcium molybdate as the final product of the furnacing operation.

8. The process of producing calcium molybdate which comprises oxidizing molybdenum sulphide to molybdenum trioxide, combining a compound containing calcium oxide available by heating with the molybdenum trioxide after the sulphur has been eliminated and effecting a reaction between the molybdenum trioxide and calcium compound to produce calcium molybdate while maintaining the mixture in the dry state.

9. The process of producing calcium molybdate which comprises roasting molybdenum sulphide to produce molybdenum trioxide, combining calcium oxide with the molybdenum trioxide after the sulphur has been eliminated and effecting a reaction between the molybdenum trioxide and calcium oxide to produce calcium molybdate while maintaining the mixture in the dry state.

10. The process of producing calcium molybdate which comprises roasting molybdenum sulphide to produce molybdenum trioxide, introducing and thoroughly intermixing an oxide of calcium with the furnace contents subsequent to the elimination of the sulphur, and effecting a reaction between the molybdenum trioxide and the calcium oxide in the roasting furnace to produce calcium molybdate.

11. The process of producing calcium molybdate which comprises roasting molybdenum sulphide to produce molybdenum trioxide, introducing a compound containing calcium oxide available by heating into the furnace subsequent to the elimination of the sulphur, thoroughly intermixing the molybdenum-trioxide and the calcium compound to prevent sublimation of the molybdenum trioxide, and adding heat to the mixture to produce calcium molybdate.

12. The process of producing calcium molybdate, consisting in roasting molybdenite, mixing the roasted product with lime, and calcining the mixture.

In testimony whereof, I have signed my name to this specification.